

July 30, 1929.

E. R. WEHR ET AL

1,722,949

METAL COATING METAL SHEETS

Filed June 1, 1926



INVENTOR  
Earl R. Wehr, Carl C. Mattie, John S. Cain

BY

Albert E. Wehr

ATTORNEYS

Patented July 30, 1929.

1,722,949

# UNITED STATES PATENT OFFICE.

EARL R. WEHR AND CARL C. MAHLIE, OF MIDDLETOWN, OHIO, AND JOHN R. CAIN, OF WASHINGTON, DISTRICT OF COLUMBIA, ASSIGNEES TO THE AMERICAN ROLLING MILL COMPANY, OF MIDDLETOWN, OHIO, A CORPORATION OF OHIO.

## METAL COATING METAL SHEETS.

Application filed June 1, 1926. Serial No. 112,866.

Our invention relates specifically to the formation of a coating on steel and iron sheets which is composed on the surface at least of an alloy of zinc and aluminum, but 5 inasmuch as certain of the steps would also be applicable to the formation of alloy coatings of different metals on metallic bodies capable of being fed through a bath, the invention has more general aspects as will subsequently appear.

In the coating of sheet metal by the method of feeding it through molten metal baths, and particularly with iron and steel, when subjected to surface treatment with metals 15 which coat the iron, the problem of securing a proper coating is rendered difficult because of the large area which must be covered, and because of the distinctness with which any defect appears on the large, smooth, flat 20 area.

It has long been considered a possible advantage in the protective coating of sheet metal, particularly iron and steel, to employ an alloy of zinc and aluminum instead of a 25 zinc spelter. The difficulties met with in such attempts as have been made in the past to use zinc aluminum instead of spelter in the usual galvanizing process are two fold. In the first place, an attempt to establish a 30 usual flux at the entrance point in the coating bath, will result in the production very rapidly of a thick, gummy product which it is impossible to employ. In the second place, those parts of the bath which are apparently 35 free of the flux, develop an improperly liquified scum, which makes it impractical to get the sheets out of the bath, using known galvanizing practice.

We have developed a process, however, 40 which takes care of these various factors, eliminates the necessity of giving more than one coating treatment, and produces a highly satisfactory product. We can, for example, produce sheets by the use of a process employing ordinary coating equipment, which 45 product is coated with pure zinc and aluminum alloyed with each other, has no spangles, can withstand all the usual bending requirements, and is practically unaffected by oven heat such as is encountered in domestic stove practice.

We accomplish our objects by that certain process to be hereinafter more specifically pointed out and claimed.

In the drawing the figure is a diagram of 55 equipment found by us to be satisfactory with our process.

We have shown a galvanizing equipment having a pot 1, with guides 2, feed rolls 3, exit rolls 4, and flux box 5. The flux box 60 should have the compartment 6 for a heat unit 7, where using pure zinc. The exit rolls have located alongside of them, any desired stirring devices that are found convenient for this purpose, such as the rolls 8, 8, which 65 operate as stirrers or agitators. A partition 9 extends down into the pot, dividing the top surface of the molten bath.

In the preferred process, pure zinc is 70 melted in the pot, and aluminum is placed in the pot, at the exit end. The aluminum alloys with the zinc, and this alloy being lighter than the zinc, stays at the surface and does not work back into the flux box. The stirring rolls are driven to keep the alloy 75 stirred and avoids improper surface conditions.

By the term pure zinc, we refer to commercially pure zinc, as distinguished from the ordinary zinc spelter, (prime western), 80 which is an alloy. Either type of zinc may be used with our process, however.

The level of zinc-aluminum alloy is indicated at 10, and the pure zinc beneath it at 11. The level of the molten zinc is shown 85 at 12, where no alloy is on its surface. The level of flux in the flux box is shown at 13.

As a flux zinc-aluminum chloride is used, together with ammonium chloride, and if some little aluminum by mischance get into 90 the flux box, it will be necessary to recondition it by the addition of hydrochloric acid to the flux box.

The cleaned metal sheet is passed through the flux into the zinc, where it becomes zinc 95 coated and thence up through the exit end of the bath, as drawn by the exit rolls, where it becomes coated with zinc-aluminum alloy.

The amount of aluminum in the floated alloy at the exit end will be maintained at 100 the desired percentage by additions of aluminum from time to time. The agitators will keep the alloy fairly uniform, and in our practice we keep the alloy at around six per cent aluminum, although this amount is not 105 essential. We find that an alloy of much less than two per cent of aluminum on the final product does not give the best results.

The final product is not spangled if pure zinc is used, but if ordinary zinc spelter (prime western) be employed, the surface will spangle unless very careful control of 5 the cooling of the sheet is exercised. However, even if the sheet does spangle, it will bend to a lapped fold (180 degrees) and will withstand oven temperatures without discoloration or deterioration.

10 While our invention has been described with reference to zinc and aluminum and was worked out with these metals in view, it would have application to other instances of 15 alloy coatings where the alloy of the lighter metal will float upon the other metal, thus preventing the transmission of the floating alloy through the bath to the flux box.

Having thus described our invention, what we claim as new and desire to secure by 20 Letters Patent, is:—

1. A process of coating ferrous sheets with zinc and aluminum which consists in passing the sheets through a flux and into a molten bath of the zinc and thence up through a 25 molten alloy of zinc and aluminum floating on the surface of the zinc.

2. A process of coating ferrous sheets with zinc and aluminum which consists in passing the sheets through a flux and into a 30 molten bath of the zinc and thence up through a molten alloy of zinc and aluminum floating on the surface of the zinc, and kept from access to the flux.

3. A process of coating ferrous sheets with

zinc and aluminum which consists in passing 35 the sheets through a flux and into a molten bath of the zinc and thence up through a molten alloy of zinc and aluminum floating on the surface of the zinc, and kept from access to the flux, and agitating 40 the said alloy.

4. A process of coating ferrous sheets with zinc and aluminum which consists in passing 45 the sheets through a flux and into a molten bath of the zinc and thence up through a molten alloy of zinc and aluminum floating on the surface of the zinc, said zinc being pure.

5. A process of coating ferrous sheets with zinc and aluminum which consists in passing 50 the sheets through a flux and into a molten bath of the zinc and thence up through a molten alloy of zinc and aluminum floating on the surface of the zinc, and kept from access to the flux, said alloy being 55 agitated and said zinc being pure.

6. A process for coating a metal body with alloys containing zinc and aluminum, which consists in passing the body through a molten flux into a molten metal body on 60 which is floating a molten alloy containing zinc and aluminum, preventing the alloy from getting into the flux and agitating the alloy, and passing the article from said metal body out through the floating alloy.

EARL R. WEHR.  
CARL C. MAHLIE.  
JOHN R. CAIN.